

Feb. 23, 1932.

J. A. KENNEDY

1,846,599

OILPROOFED ELECTRICAL CONDUIT, INSULATION, ETC

Filed Dec. 15, 1928



Fig. 1.



Fig. 2.

Inventor  
Joseph A. Kennedy  
Usina & Rauber  
Atlys

## UNITED STATES PATENT OFFICE

JOSEPH A. KENNEDY, OF PAWTUCKET, RHODE ISLAND, ASSIGNOR, BY MESNE ASSIGNMENTS, TO ANACONDA WIRE AND CABLE COMPANY, A CORPORATION OF DELAWARE

## OILPROOFED ELECTRICAL CONDUIT, INSULATION, ETC.

Application filed December 15, 1928. Serial No. 326,411.

The present invention relates to protective coverings or jackets for electrical conductors, whether constructed and applied directly about a bare or an insulated wire as an inseparable envelope, or made as an open tube or conduit adapted to be passed over, or to receive, a bare or covered wire or cable; and it is particularly concerned with flexible jackets made of fibrous strands interconnected or interlocked by weaving, braiding, knitting, or otherwise. The object of the invention is to give to protecting means of the character indicated not only water-resistant and flame-resistant qualities suitable for the requirements of the art, but oil-resistant qualities as well.

The invention will be fully apparent from the following specification and will be defined with particularity as required by the statutes in the appended claims.

One embodiment of the invention is exemplified in Fig. 1 which is an elevation of an electrical conductor with portions broken away to reveal interior portions.

Fig. 2 exemplifies the invention embodied in a conduit adapted to be passed over, or to receive, a bare or covered wire cable.

In the embodiment illustrated in Fig. 1, 10 are conductors, each of which are covered 30 with a water-proofing coating 12 such as asphaltum. This coating is in turn covered with a flexible jacket 14 which has a covering of a flame-proofing compound such as stearin pitch impregnated therein. Over 35 this layer, there is applied, in a manner hereinafter described, a film or coating of a substance which is insoluble in solvents of the stearin pitch. While not limited thereto this insoluble coating of film may constitute a

40 homogeneous or continuous film of sodium silicate which can be conveniently applied in the form of an aqueous solution. If desired, this solution may be impregnated in an outer jacket 16. Over the layer or film of sodium silicate, there is applied a thin layer or coating of cellulosic lacquer. As shown in Fig. 1, 45 a pair of cables having the protective coating herein described may be enclosed in an outer sheath comprising the layers *a*, *b*, *c* and *d*. 50 The innermost layer *a* being impregnated or

coated with a water-proofing compound such as asphaltum or the like to which is applied a layer of flame-proofing material indicated at *b*. Over this there is a layer of sodium silicate or similar material which is insoluble in the solvent in the flame-proofing material. Over the layer *c*, there is applied a layer *d* of suitable lacquer having oil resisting properties.

Fig. 2 illustrates the invention applied to a hollow tube or conduit having layers *a*, *b*, *c* and *d* which are substantially the same as the correspondingly identified layers of Fig. 1.

In carrying the invention into effect, I first treat the protecting jacket with a water-proofing compound or agent; preferably using asphaltum for this purpose, although I do not limit myself to that specific material. The asphaltum or other water-proofing substance may be applied in either melted condition or in solution with a volatile solvent in any known or other suitable manner. I next apply to the outer surface of the protective jacket a coating of flame-proofing compound, preferably stearin pitch rendered fluid by heat; although here again I am not narrowly limited to a specific material. The above named compounds have long been known and commonly used for treating both open conduits formed of interwoven flexible strands and conductors and cables on which fibrous braided, knitted or woven jackets have been built. They may be applied for the purposes of the present invention by immersing the fabric in tanks containing the fluid compounds, or in any other manner already known or which may be hereafter devised.

In the further carrying out of the invention, the treated jacket or jacketed conductor is coated with sodium silicate, preferably by being drawn through a tank containing a freely flowing aqueous solution of sodium silicate. The viscosity of the solution may vary within relatively wide limits, from that of a thin syrup little more viscous than water, to a viscosity approximating that of molasses. The excess of solution is wiped from the article as the latter passes out of the tank

55

60

65

70

75

80

85

90

95

100

and the adherent film is allowed to dry, either by exposure to the surrounding air for a sufficient length of time, or more rapidly by passing through a heated oven or in exposure to other suitable heating means.

5 When the film of sodium silicate is sufficiently firm, the oil-proofing treatment is carried out by coating the article with cellulosic lacquer, as nitrocellulose, cellulose acetate, or other cellulose compound which is capable of being provided in dissolved condition and has the desired oil-resistant properties. Inasmuch as it is desirable to produce the finished article at as low cost as 10 possible, I prefer to use the least expensive compounds of cellulose and solutions of such compounds which will serve the purpose. From this point of view, nitrocellulose is preferable to other cellulosic compounds, and 15 the less expensive of the known suitable solvents of nitrocellulose are used to dissolve it and to dilute the solution. Any of the known softeners or emollients for cellulosic compounds may be included in the lacquer 20 in order that the coating when dried may be sufficiently elastic and flexible. The lacquer is likewise preferably applied by passing the conduit or jacketed conductor through a body of the lacquer solution in a 25 tank, wiping off the excess as the article emerges from the tank, and drying the residual film. Two or more such films may be thus applied in succession in order to build up a coating of the required thickness. This 30 lacquer coating step is the final step in producing the finished article.

The jacket thus produced is resistant to penetration by water and oil and to ignition by flame. Preferably the initial water-proofing compound is applied in such a way as substantially to saturate the constituent strands so that they will not absorb moisture either from water coming into direct contact with the structure or from vapor in the 40 atmosphere. Both the flame-proofing coat of stearin pitch and the lacquer coat are also impervious to water and form external water-repellent means; the lacquer coat also protecting the film of sodium silicate from attack and dissolution by water. Both the film of sodium silicate and the outer coat of lacquer protect the jacket against attack by oil, which is a solvent of asphaltum, stearin pitch and other hydrocarbonaceous materials 45 used for initial water-proofing and flame-proofing. Thus my improved jackets are suitable to protect electrical conductors used in automobiles in the vicinity of the engine, or other situations where they are liable to 50 be spattered or covered with oil.

While some cellulose compounds which may be used as the basis of oil-resistant lacquer are relatively non-inflammable, others, including nitrocellulose, are highly 55 inflammable. However, even nitrocellulose

used in this environment does not constitute a fire hazard because it is applied in such a thin coat that, even if ignited, it does not generate enough heat to have any effect on the flame-proofing compound.

The flame-proofing effect given by stearin pitch is augmented and enhanced by the film of sodium silicate on the pitch coating. The value of stearin pitch as a flame-proofing agent arises from the fact that, although it is 60 not incombustible, it nevertheless contains but a small proportion of inflammable matter and is ignited only with difficulty, and when ignited it quickly forms a porous or blister-like ash imprisoning inert gases which have 65 heat insulating effect about the enclosed conductors and the inflammable insulation thereof. And even when the pitch coating is ignited in one part of the fabric by intense heat, the flame is soon extinguished and does 70 not travel along the jacket from the heated part. But even such slight combustion as stearin pitch undergoes when exposed to flame is largely prevented by the outer film of sodium silicate, which is wholly incombustible and excludes air from the enclosed stearin pitch.

In addition to its oil-proofing and flame-proofing qualities above described, the sodium silicate film likewise protects the asphaltum 75 and flame-proofing compound from attack by the solvents in the lacquer solution. Many of the solvents of nitrocellulose will dissolve stearin pitch, and the lacquer solutions and thinners which I prefer to use on account of 80 their low price have so powerful a solvent action on stearin pitch that the latter is liable to be softened by the solvents and impermeated by the nitrocellulose, during its immersion in the lacquer bath, to such an 85 extent as to diminish seriously its flame-proofing capacity. But sodium silicate is insoluble in the lacquer solvents and wholly protects all parts of the stearin pitch coat 90 which it covers from attack by these solvents.

However, it is desirable to effect a commingling to some extent of the lacquer coating with the pitch coating in order to anchor the lacquer coating firmly to the jacket so that it cannot be readily peeled off if it should be injured by abrasion. Hence I prefer to apply the sodium silicate in such a thin solution, or wipe off so much of the adherent solution while still wet that the high points of the jacket will be bare of the silicate and hence subject to attack by the lacquer solvents. Fabricated jackets of the type with which this invention is particularly concerned are more or less rough on the outside where their interconnected strands cross one another, and such roughness remains in some measure after the fabric has emerged from the flame-proofing bath. Hence by wiping it when it leaves the bath of sodium silicate solution, the high points are left with little or no sodium sili-

- cate upon them. The stearin pitch at these points is softened by the lacquer solvents and becomes interlocked and bonded with the lacquer coating when the latter has dried. 5 Thus the lacquer coat is securely attached to the fabric at discontinuous points while being excluded from penetration into the stearin pitch coat over most of the surface of the fabric.
- 10 While the article thus described in detail is the preferred embodiment of the invention, modifications and variations may be made without departing from the spirit of the invention or the scope of the appended claims.
- 15 For instance, the entire surface of the stearin pitch coating may be covered with sodium silicate if it is desired to extend the flame-proofing qualities imparted by the latter to all points.
- 20 The term "jacket" as used in this specification is intended to include both independent conduit or tubing adapted to receive conductors, and envelopes formed originally upon insulated wires or cables and embracing the same so closely as to be practically immovable thereon. An illustration of a suitable structure for such jackets is given by the patent to Charles S. Smith, No. 1,016,527, February 6, 1912. However, the invention is not limited to jackets of this particular construction but includes those made of any other materials and in any other way which may be advantageously treated in accordance with the principles hereinbefore described.
- 25 What I claim and desire to secure by Letters Patent is:
1. A jacket for the protection of electrical conductors having a flame-proofing coat, an outer oil-proofing coat, and an intermediate homogeneous coat of a substance which is insoluble by the solvents of the flame-proofing and oil-proofing coats.
  2. A protective jacket for electrical conductors having a flame-proofing coat, an outer coat of oil-proofing material bonded at separated points to the flame-proofing coat, and an intermediate homogeneous film of material which is insoluble in the solvents of the before named coats interposed between said coats where the latter are not thus bonded together.
  3. A protective jacket for electrical conductors having a flame-proofing coat of stearin pitch, an outer coat of cellulose lacquer, and an intermediate coat of sodium silicate.
  4. A protective jacket for electrical conductors having a protective coating, an outer coat of oil-proof lacquer and an intermediate film of a substance which is insoluble by the solvents of the first named coat.
  5. A coated jacket for electrical conductors having coatings of different materials, comprising an outermost oil-proof coat which is the residue of an originally fluid solution, an innermost coat which is a substance somewhat soluble in the solvent of said solution, and an intermediate homogeneous coat comprising a substance which is insoluble by the solvent of the substance which forms the outermost coat.
6. A protective jacket for electrical conductors having a flame-proofing coat of stearin pitch, an outer coat of cellulose lacquer, and an intermediate coat of sodium silicate, said intermediate coat being penetrated at isolated points by the stearin pitch coat, and the said coats of stearin pitch and lacquer being bonded together by commingling at such points.
7. A water-, oil-, and flame-resistant protective jacket for electrical conductors comprising a fabric having an impregnation of asphaltum, a coat of stearin pitch on its exterior, a film of sodium silicate outside of the last named coat, and a coat of cellulose lacquer outside of all.
8. The method of flame-proofing and oil-proofing protective jackets of and for electrical conductors which comprises coating the jacket with a flame-resistant compound, applying on said compound an aqueous coating of non-combustible material which is insoluble by the common solvents of the flame-proofing coat and the after mentioned oil-proofing coat, and finally applying an outer coat of a lacquer which is insoluble in oil, in solution with a volatile solvent, and drying said outer coat.
9. The method of flame-proofing and oil-proofing protective jackets of and for electrical conductors which comprises coating the jacket with a flame-resistant compound, applying on said compound an aqueous solution and drying it to form a coat of non-combustible material which is insoluble by the common solvents of the flame-proofing coat and the after mentioned oil-proofing coat in such manner that isolated points of the first coat are substantially free from the material of the second coat, and applying an outer coat of lacquer in solution with a solvent which is also a solvent of the first named coat, whereby the lacquer becomes commingled and bonded with the first coat at the points which are not covered by the second coat, said lacquer being insoluble by oil.
10. The method of oil-, water-, and flame-proofing jackets of and for electrical conductors which comprises coating the conductor with liquefied stearin pitch, applying an aqueous solution of sodium silicate upon said stearin pitch coat, drying such solution, and finally applying cellulose lacquer dissolved in a volatile solvent to the jacket and drying the lacquer coat.
11. The method of oil-, water-, and flame-proofing jackets of and for electrical conductors which comprises coating the jacket with melted stearin pitch, applying a water solution of sodium silicate outside of the stearin

pitch coating and leaving isolated points of the latter uncovered by said solution, drying the sodium silicate coat, and finally coating the jacket with a cellulose compound in solution with a solvent which is also a solvent of stearin pitch, and drying the last named coat.

In testimony whereof I have affixed my signature.

10

JOSEPH A. KENNEDY.

15

20

25

30

35

40

45

50

55

60